

# United States Patent Office

3,156,595

Patented Nov. 10, 1964

1

3,156,595

## CHEMICAL COMPOSITION FOR PRODUCING HEAT

Albert T. Camp and Gerald L. MacKenzie, Redlands, Calif., assignors, by mesne assignments, to Lockheed Aircraft Corporation, Burbank, Calif., a corporation of California

No Drawing. Filed Sept. 21, 1961, Ser. No. 139,613

5 Claims. (Cl. 149—87)

The present invention relates to compositions of matter which react to produce heat, and the primary object of the invention is to provide a fluid composition which, when dispensed onto a hot surface, reacts exothermically without appreciable gaseous by-products. Thus, the composition of the present invention is adapted for use in a closed system where it would be inconvenient or impossible to dispose of combustion products.

Another object of the invention is to provide a completely self-contained composition that reacts with the evolution of large quantities of heat without consuming oxygen which may be in limited supply, as in a submarine or space capsule. A typical application of the present invention would be for under-sea power supply packages, in which the heat output of the composition is converted to electricity for the purpose of charging batteries by means of the Peltier principle, using a thermopile, or by thermionic conversion systems.

A further object of the invention is to provide a chemical composition for producing heat, which is chemically stable up to 400° F., and which is non-explosive.

One important advantage of the present invention is that on the basis of energy production, the fluid compositions of the invention provide more heat per unit of volume than any known common propellant or explosive, and, in, fact, provide among the highest outputs known in the chemical energy field. This fact, coupled with its high stability and gaslessness, make the compositions of the present invention useful for the generation of heat in closed systems.

In a broad form of the invention, our heat-producing composition consists of a fluid slurry of active, finely powdered metals selected from the group consisting of lithium, aluminum, magnesium, sodium, potassium, rubidium, caesium and beryllium, or alloys thereof, suspended in a fluorochlorocarbon oil, such as Kel-F, manufactured by Minnesota Mining & Mfg. Co., or Fluorolube, manufactured by Hooker Electrochemical Corp. Preferably, the powdered metal includes a minor proportion of lithium, either as a pure metal or in the form of an alloy with one of the other metals named; in which the lithium constitutes approximately 3% to 4% of the total weight of the composition, while the other metal or metals constitutes approximately 21% to 22% of the total weight, and the fluorochlorocarbon oil constitutes approximately 75% of the weight. The lithium, being an extremely active metal, tends to react first with the fluorochlorocarbon oil, and the heat of its reaction serves to initiate the reaction of the less reactive metal.

The exact structure of the fluorochlorocarbon oil is somewhat variable, and is generally shown as  $(C_2F_3Cl)_n$ , wherein the subscript  $n$  represents the number of molecules linked together to form a chain. These fluorochlorocarbon oils have densities ranging from 1.8 to 2.1, and therefore in order to maintain a stable dispersion of finely powdered metal in the oil, it is necessary that the metal or alloy be of approximately the same density as the oil. Aluminum is the preferred major constituent of the powdered metals because the density of its alloys useful for this application approximates that of the fluorochlorocarbon oil. Since lithium is the lightest metal

2

known, with a specific gravity of only 0.53, it is preferable to use an alloy of lithium and aluminum, or lithium and one of the other metals in the group named hereinbefore. The incorporation of 0.2% to 0.3% of a very fine silica, in the range of 0.01 to 0.03 micron particle size improves the combustion efficiency and retards settling of the metal.

### Example 1

A fluid slurry consisting of 75% by weight of fluorochlorocarbon oil, 22% by weight of finely powdered aluminum, and 3% by weight of finely powdered lithium, was thoroughly mixed to produce a uniform dispersion. This slurry was dispensed slowly onto a hot surface at 600° F., with the following dual reaction:



The above two reactions are exothermic, and the amount of heat given off by the reactions is expressed by the following thermochemical equations, where the molar energies represent heats of formation of the reactants and products:



Heat of reaction (1) = 565 kcal./mol

The atomic weights of the elements involved in the above reaction are:

$$C = 12.01$$
$$F = 19.00$$
$$Cl = 35.46$$
$$Al = 26.98$$

The gram molecular weights of the fluorochlorocarbon oil and aluminum entering into the reaction are as follows:

$$3(C_2F_3Cl) + 4Al$$
$$349.44 \text{ gms.} + 107.92 \text{ gms.} = 457.36 \text{ gms.}$$
$$457.36 \text{ gms. yields } 565 \text{ kcal.}$$

Converting from kcal./mol to cal./gm. gives:

$$565 \text{ kcal./mol} = 1235 \text{ cal./gm.}$$

The thermochemical reaction of lithium with fluorochlorocarbon oil is as follows:



Heat of reaction (2) = 338.45 kcal./mol

The molecular weight of Li is 6.94, and the gram molecular weights of the fluorochlorocarbon oil and lithium entering into the reaction are as follows:

$$C_2F_3Cl + 4Li$$
$$116.46 \text{ gms.} + 27.76 \text{ gms.} = 144.22 \text{ gms.}$$
$$144.22 \text{ gms. yields } 338.45 \text{ kcal.}$$

Converting from kcal./mol to cal./gm. gives:

$$338.45 \text{ kcal./mol} = 2341 \text{ cal./gm.}$$

As there is roughly seven times as much aluminum by weight as there is lithium in the composition, the combined heat of the reaction between the two metals and the fluorochlorocarbon oil is approximately 1275 calories per gram of lithium/aluminum/fluorochlorocarbon slurry.

## Example 2

A slurry of finely divided lithium/aluminum alloy was dispersed in fluorochlorocarbon oil, at the ratio of 25 parts by weight of alloy to 75 parts by weight of fluorochlorocarbon oil. The alloy consisted of 14.8% by weight of lithium, and 85.2% by weight of aluminum. Thus, the lithium is 3.7% of the total formulation. Dispensed dropwise onto a hot plate, the chemical reaction is substantially the same as in Example 1, except that a somewhat higher heat output of 1399 cal./gm. is obtained, due to the higher content of lithium.

## Example 3

A slurry was prepared by dispersing a finely divided ternary alloy of lithium, magnesium and aluminum, together with a small quantity of colloidal silica ranging in particle size from 0.01 to 0.03 microns, in fluorochlorocarbon oil in the proportions of 25% by weight of alloy, 74.8% fluorochlorocarbon oil, and 0.2% colloidal silica. The alloy consisted of 10% by weight of lithium, 18% magnesium, and 72% aluminum. When dispensed dropwise on a hot plate of over 600° F., the slurry reacted thermochemically, with the evolution of large quantities of heat without appreciable gaseous by-products.

The reaction of the lithium and aluminum in the alloy with the fluorochlorocarbon oil is as given in Example 1, while the thermochemical reaction of the magnesium with the fluorochlorocarbon oil is as follows:



The molecular weight of Mg is 24.32, and the gram molecular weights of the fluorochlorocarbon oil and magnesium entering into the reaction are as follows:



Converting from kcal./mol to cal./gm. gives:

$$551 \text{ kcal./mol} = 1670 \text{ cal./gm.}$$

The colloidal silica does not enter into the reaction, but retards settling of the alloy and improves combustion efficiency.

Obviously, many modifications and variations of the invention as hereinbefore set forth may be made without departing from the spirit and scope thereof, and therefore only such limitation should be imposed as are indicated in the appended claims.

We claim:

1. A composition for producing heat without appreciable gaseous by-products when dispensed drop-wise onto a hot surface, said composition consisting of a fluid slurry

of finely divided metals in a fluorochlorocarbon oil containing fluorine, chlorine, and carbon atoms in the approximate ratios shown by the formula  $C_2F_3Cl$ , said metals consisting of lithium in the proportion of about 3% to 4% of the total weight and aluminum in the proportion of about 21% to 22% of the total weight.

2. A composition for producing heat without appreciable gaseous by-products when dispensed dropwise onto a hot surface, said composition comprising a fluid slurry of a finely divided metal in a fluorochlorocarbon oil containing fluorine, chlorine, and carbon atoms in the approximate ratios shown by formula  $C_2F_3Cl$ , said metal consisting of a lithium/aluminum alloy in which lithium is about 15% by weight of the total metal, and the remainder is aluminum, said finely divided metal being in the proportion of about 25% of the total weight of the composition, and said fluorochlorocarbon oil being in the proportion of about 75% of the total weight.

3. A composition for producing heat without appreciable gaseous by-products when dispensed onto a hot surface having a temperature above 600° F., said composition comprising a fluid slurry consisting of about 25% by weight of a finely divided ternary alloy of lithium, magnesium and aluminum, together with about 0.2% of colloidal silica dispersed in a fluorochlorocarbon oil containing fluorine, chlorine, and carbon atoms in approximate ratios shown by the formula  $C_2F_3Cl$ , said alloy consisting of about 10% by weight of lithium, about 18% magnesium, and about 72% aluminum.

4. A fluid composition for producing heat without gaseous by-products when ignited in a closed system, said composition consisting of an alkali metal selected from the group consisting of lithium, sodium, and potassium; a light metal selected from the group consisting of aluminum, magnesium, and beryllium; and a fluorochlorocarbon oil containing fluorine, chlorine, and carbon atoms in the approximate ratios shown by the formula  $C_2F_3Cl$ , said alkali and light metals together constituting about 25% of the total weight.

5. A fluid composition for producing heat without gaseous by-products when ignited in a closed system, said composition consisting of about 3% to 4% by weight of lithium; about 21% to 22% by weight of a light metal selected from the group consisting of aluminum, magnesium, and beryllium; and the remainder of a fluorochlorocarbon oil containing fluorine, chlorine, and carbon atoms in the approximate ratios shown by the formula  $C_2F_3Cl$ .

## References Cited in the file of this patent

## UNITED STATES PATENTS

1,318,074 Gowdy ----- Oct. 7, 1919

## FOREIGN PATENTS

127,031 Great Britain ----- May 29, 1919